

Patented May 14, 1935

2,001,385

# UNITED STATES PATENT OFFICE

2,001,385

## ELECTROLYTIC DEPOSITION OF NICKEL FROM NICKEL SALT SOLUTIONS

Anton Martin Grønningssæter, New York, N. Y.,  
assignor to Falconbridge Nickel Mines Limited,  
Toronto, Ontario, Canada

No Drawing. Application August 15, 1933, Serial  
No. 685,224. In Norway August 27, 1932

3 Claims. (Cl. 204—14)

This invention relates to the electrolytic deposition of nickel from nickel salt solutions as employed in the metallurgy of nickel.

In the usual processes of electrolytic refining of metals, the deposition of the metal is frequently effected on so-called "starting" sheets or plates of the same metal as that to be deposited. Such starting sheets are employed for example in the refining of copper, lead and nickel. In these known processes these "starting" sheets have not been subjected to any preparatory treatment; and as a matter of fact such preparatory treatment has for instance for copper not been found necessary.

However, as regards nickel, the practice hitherto followed entails considerable disadvantages. Thus it frequently happens that the deposited nickel flakes off from the starting sheets already in the deposition tanks, which causes short circuiting and other difficulties, particularly noticeable when refining according to the well-known Hybinette process with the cathodes placed in the "Hybinette bag".

In the course of the subsequent cutting of the nickel cathodes into smaller pieces, splitting of the deposited nickel from the starting sheet usually takes place. This splitting causes considerable drawbacks.

Difficulties of a similar kind are experienced also in the art of electroplating. In this art it is frequently difficult to make the deposited metal adhere firmly to the metal to be covered. In order to overcome these difficulties, various means, such as for example grinding, treatment with alkaline liquors, comparatively strong acids and the like, have been tried, with more or less satisfactory results. These known means have been considered of little use or too expensive in connection with the refining of nickel.

The present invention has for its object a method for treating starting sheets of nickel, whereby it is made possible to avoid the flaking and splitting above referred to. This result is obtained in a simple and inexpensive way by subjecting the starting sheets prior to their use to the action of a dilute acid, for example sulphuric acid for some time. The acid is preferably employed in a warm condition and may be highly diluted.

Thus by the use of sulphuric acid, satisfactory results have been obtained by treating the sheets for a few hours with an acid containing not more than 1% concentration, 10 g. H<sub>2</sub>SO<sub>4</sub> in the liter.

In practice it has been found unnecessary to wash the prepared starting sheets before use;

on the contrary, the small amounts of dilute acid adhering is an advantage. It has been found that immediate introduction in the deposition tanks is not necessary, so that a considerable number of prepared starting sheets, for instance about the thirty to sixty plates usually needed for one or two deposition tanks can be removed from the pickling tank at a time.

The preparatory acid treatment of the nickel sheets is suitably carried into effect by placing the sheets in tanks containing dilute sulphuric acid which is kept in continuous motion by blowing with steam or air or by other suitable means. In these acid tanks the "starting" sheets are submerged some time before they are to be used in the deposition tanks, for example the evening before such use and removed as needed during the next day.

The preparatory treatment is entirely efficient and requires little manual labour and inspection.

The method is of considerable practical importance in the usual electrolytic refining of nickel and is particularly advantageous when the resulting nickel cathodes are to be used as anodes in the nickel plating industry, in which case it is highly important to avoid splitting of the anodes during preparation or use.

The practice of the invention may be better understood by a consideration of the following example:

Nickel is deposited electrolytically on aluminum mother plates and stripped when of desired thickness, for use as nickel starting sheets. 400 to 500 such starting sheets are used at the present time every day at the refinery where this method was worked out. The starting sheets are placed in the pickling bath with about 1% sulphuric acid and generally kept for several hours; the temperature is kept at about 50° C. 40 by direct or indirect steam heating. During the treatment the bath is kept in circulation by blowing in air in order to renew the acid at the surface of the starting sheets and in order to keep a uniform temperature of the electrolyte. 45 The treatment generally lasts for 12 hours. 70 starting sheets are removed at a time from the bath and are then in the course of about half an hour placed in the deposition tanks.

I claim:

1. In the electrolytic refining of nickel when using deposition of nickel on nickel starting sheets, the method which consists in subjecting the starting sheets prior to being introduced into the electrodeposition cell to the action of dilute

50

55

acid of sufficient strength to effect dissolution of basic nickel compounds on the surface of the sheets but so dilute as not to attack to any appreciable extent the metallic nickel even when left in contact with the metal for several hours.

2. Process according to claim 1, in which nickel starting sheets after having been subjected to the preparatory treatment in dilute

acid are introduced into electrodeposition cells while still moist with the adhering acid.

3. Process according to claim 1, in which the preparatory treatment of the starting sheets takes place in warm sulphuric acid of no more than about 1% concentration.

ANTON MARTIN GRÖNNINGSÆTER.